

# United States Patent [19]

Kablaoui

[11] 4,231,758  
[45] Nov. 4, 1980

[54] MOTOR FUEL COMPOSITION

[75] Inventor: Mahmoud S. Kablaoui, Wappingers Falls, N.Y.

[73] Assignee: Texaco Inc., White Plains, N.Y.

[21] Appl. No.: 698,436

[22] Filed: Jun. 21, 1976

[51] Int. Cl.<sup>3</sup> ..... C10L 1/22

[52] U.S. Cl. ..... 44/71; 44/70

[58] Field of Search ..... 44/71, 70, 58

[56] References Cited

U.S. PATENT DOCUMENTS

|           |         |              |       |
|-----------|---------|--------------|-------|
| 2,844,449 | 7/1958  | Dille et al. | 44/70 |
| 3,773,479 | 11/1973 | Dorn et al.  | 44/71 |
| 3,901,665 | 8/1975  | Polss        | 44/58 |
| 3,909,214 | 9/1975  | Polss        | 44/58 |

Primary Examiner—Winston A. Douglas

Assistant Examiner—Mrs. Y. Harris-Smith

Attorney, Agent, or Firm—Carl G. Ries; Robert A. Kulason; James J. O'Loughlin

[57] ABSTRACT

Motor fuel composition comprising a mixture of hydro-

carbons in the gasoline boiling range containing in combination a minor amount of a substituted asparagine containing the formula:



in which R and R' each represent a secondary or tertiary alkyl or alkylene radical having from about 7 to about 20 carbon atoms and a minor amount of a carboxylic acid ester having the formula:



in which R is a divalent aliphatic hydrocarbon radical, containing 2 to 10 carbon atoms, R' is hydrogen or an aliphatic hydrocarbon radical containing 2 to 18 carbon atoms, x has a value from 1 to 4 and n has a value from 0 to 4.

9 Claims, No Drawings



bonate), diethylene glycol bis (ethoxyethyl carbonate), diethylene glycol bis (propoxyethyl carbonate), diethylene glycol bis (hexoxyethyl carbonate), diethylene glycol bis (octoxyethyl carbonate), propylene glycol bis (butoxyethyl carbonate), dipropylene glycol bis (ethoxyethyl carbonate), diethylene glycol bis (pentoxyethyl carbonate), tetraethylene glycol bis (ethoxyethyl carbonate), tri-ethylene glycol bis (butoxyethyl carbonate), tetraethylene glycol bis (propoxyethyl carbonate), triethylene glycol bis (octoxyethyl carbonate), triethylene glycol bis (butoxyethyl carbonate), diethylene glycol (bis-n-pentoxyethoxyethyl carbonate) and tetraethylene glycol bis (2-ethylhexoxyethyl carbonate).

The motor fuel composition of the invention comprises a mixture of hydrocarbons boiling in the gasoline boiling range i.e. generally from about 85° to 450° F.

The gasoline motor fuel which is benefitted by the novel detergent additive combination of the invention may be leaded or unleaded and may consist of straight chain or branched-chain paraffins, cycloparaffins, olefins and aromatic hydrocarbons and mixtures of these. The base fuel can be derived from straight run naphtha, polymer gasoline, natural gasoline or from catalytically cracked or thermally cracked hydrocarbons and catalytically reformed stocks. The hydrocarbon composition and the octane level of the base fuel are not critical. Any conventional motor fuel base may be employed in the practice of this invention.

In general, the additive components of the invention are added to a fuel composition in minor amounts, i.e., amounts effective to cooperate in providing the enhanced detergency of the fuel composition. The substituted asparagine additive is employed in an amount ranging from about 0.001 to 5.0 weight percent based on the total fuel composition with an amount ranging from about 0.001 to 0.2 weight percent being preferred. The most effective concentration of this additive component ranges from about 0.002 to 0.10 weight percent.

The carbonate acid ester compound which was discovered to cooperate with the substituted asparagine compound is employed in an amount ranging from about 0.01 to 0.05 volume percent of the finished fuel composition. The preferred concentration of this additive component is from about 0.05 to 0.25 volume percent of the gasoline composition.

A fuel composition containing the additive combination of the invention can contain other additives normally employed in a gasoline motor fuel composition. For example, the base fuel may be blended with an anti-knock compound, such as tetraethyl lead compound, including tetraethyl lead, tetramethyl lead, tetrabutyl lead, or mixtures thereof generally in a concentration from about 0.01 to 4.0 cc. per gallon of gasoline. The tetraethyl lead mixture commercially available for automotive use will also contain an ethylene chloride-ethylene bromide mixtures as scavenger for removing lead combustion products from the engine. The fuel composition may also be augmented with anti-icing additives, corrosion inhibitors, dispersants and upper cylinder lubricants.

The additive combination of the invention was tested for its effectiveness as a carburetor detergent in the Buick Carburetor Detergency Test. This test is run on a Buick 350 CID V-8 Engine equipped with a two-barrel carburetor. The engine is mounted on a test stand and has operating EGR and PCV systems. The test cycle, shown in Table I, is representative of normal road oper-

ation. Approximately 300 gallons of fuel and three quarts of oil are required for each run.

Prior to each run the carburetor is completely reconditioned. Upon completion of the run, the throttle plate deposits and the deposits on the area below the throttle plate are visually rated according to a CRC Varnish rating scale (Throttle Plate Merit Rating) where a rating of (1) one describes heavy deposits on the throttle plate and a rating of (10) ten a completely clean plate. The two ratings are averaged to give an average carburetor rating.

TABLE I

| 1973 BUICK CARBURETOR DETERGENCY TEST OPERATING CONDITIONS |             |           |           |
|------------------------------------------------------------|-------------|-----------|-----------|
|                                                            | Stage I     | Stage II  | Stage III |
| Duration, hour                                             | 1           | 3         | 1         |
| Speed, r.p.m.                                              | 650 +<br>25 | 1500 + 25 | 2000 + 25 |
| Torque, ft. lbs.                                           | 0           | 80 + 2    | 108 + 2   |
| Water Out, °F.                                             | 205 + 5     | 205 + 5   | 205 + 5   |
| Carburetor Air, °F.                                        | 140 + 5     | 140 + 5   | 140 + 5   |
| Exhaust Back Pres. in Hg.                                  | —           | 0.7 + 0.1 | —         |
| Man. Vac., In Hg.                                          | 18-20       | 14-17     | 11-13     |
| Fuel Flow, lbs/hr.                                         | ~4          | ~14       | ~20       |
| Test Duration, 120 hours                                   |             |           |           |

The fuel composition employed for testing the detergent additive combination of the invention was an unleaded gasoline base fuel having a Research Octane Number of 96. This gasoline consisted of about 23% of aromatic hydrocarbons, 12% olefinic hydrocarbons and 65% paraffinic hydrocarbons and boiled in the range from 94° to 377° F.

Test results obtained employing the detergent additive combination of the invention and comparison test results are given in the Table below.

TABLE II

| BUICK CARBURETOR DETERGENCY TEST |                                                                                                                                                                    |                   |
|----------------------------------|--------------------------------------------------------------------------------------------------------------------------------------------------------------------|-------------------|
| Run                              | Fuel                                                                                                                                                               | Carburetor Rating |
| 1.                               | Unleaded Base Fuel                                                                                                                                                 | 3.0               |
| 2.                               | Unleaded Base Fuel + PTB N,N'-di-C <sub>15</sub> -C <sub>20</sub> secondary alkyl asparagine <sup>2</sup>                                                          | 5.0               |
| 3.                               | Unleaded Base Fuel + 200 PTB of diethylene-bis-2-ethoxyethyl carbonate                                                                                             |                   |
| 4.                               | Unleaded Base Fuel + 15 PTB N,N'-di-C <sub>15</sub> C <sub>20</sub> secondary alkyl asparagine + 200 PTB diethyleneglycol-bis-2-ethoxyethyl carbonate <sup>2</sup> | 6.4               |
| 5.                               | Unleaded Base Fuel + 15 PTB N,N'-di-C <sub>15</sub> -C <sub>20</sub> secondary alkyl asparagine + 200 PTB diethyleneglycol-bis-hexyl carbonate <sup>2</sup>        | 6.3               |

<sup>(1)</sup>PTB = Pounds of additive per 1000 barrels of fuel

<sup>(2)</sup>These fuels also contained 18 PTB of a corrosion inhibitor and 43 PTB of a carrier mineral oil.

Run 3 shows that a carbonate acid ester has absolutely no effect on the carburetor detergency of a motor fuel composition. In contrast, Runs 4 and 5, containing a carbonate acid ester in combination with a substituted asparagine provided a substantial improvement in carburetor detergency over Run 2 which contained the substituted asparagine without the carbonate acid ester. These results were unexpected in view of the absence of carburetor detergency in carbonate acid ester alone.

I claim:

1. A motor fuel composition comprising a mixture of hydrocarbons in a gasoline boiling range containing from about 0.001 to 5.0 weight percent of a substituted asparagine having the formula:



in which R and R' each represent a secondary or a tertiary alkyl or alkylene radical having from about 7 to 20 carbon atoms and from about 0.01 to 0.05 volume percent of a carbonic acid ester having the formula:



in which R is a divalent aliphatic hydrocarbon radical containing 2 to 3 carbon atoms, R' is hydrogen or an aliphatic hydrocarbon radical containing 2 to 18 carbon atoms, x has a value from 1 to 4 and n has a value from 0 to 4.

2. A motor fuel composition according to claim 1 in which R and R' in said substituted asparagine represent secondary hydrocarbyl radicals.

3. A motor fuel composition according to claim 1 in which said substituted asparagine is N,N'-di-C<sub>15</sub>-C<sub>20</sub> secondary alkyl asparagine.
4. A motor fuel composition according to claim 1 in which said substituted asparagine is N,N'-di-C<sub>11</sub>-C<sub>14</sub> secondary alkyl asparagine.
5. A motor fuel composition according to claim 1 in which said carbonic acid ester is a glycolbis (glycol ether carbonate).
- 10 6. A motor fuel composition according to claim 1 in which said carbonic acid ester is diethylene glycol-bis-2-ethoxyethyl carbonate.
7. A motor fuel composition according to claim 1 in which said carbonic acid ester is diethyleneglycol-bis-hexyl carbonate.
- 15 8. A motor fuel composition according to claim 1 containing from about 0.001 to 0.2 weight percent of said substituted asparagine and from about 0.05 to 0.25 volume percent of said carbonate acid ester.
- 20 9. A motor fuel composition according to claim 1 in which said hydrocarbon mixture boils in the range from about 85° to 450° F.

\* \* \* \* \*

UNITED STATES PATENT AND TRADEMARK OFFICE  
CERTIFICATE OF CORRECTION

PATENT NO. : 4,231,758

DATED : November 4, 1980

INVENTOR(S) : Mahmoud S. Kablaoui

It is certified that error appears in the above-identified patent and that said Letters Patent is hereby corrected as shown below:

Column 5, line 8, "0.05" should read --0.5--.

Signed and Sealed this

*Eleventh Day of August 1981*

[SEAL]

*Attest:*

GERALD J. MOSSINGHOFF

*Attesting Officer*

*Commissioner of Patents and Trademarks*